

# UNITED STATES PATENT OFFICE.

FRITZ WIEDERMANN, OF CHARLOTTENBURG, GERMANY, ASSIGNOR TO THE FIRM OF  
"VEREINIGTE CHEMISCHE WERKE" ACTIENGESELLSCHAFT, OF CHARLOTTEN-  
BURG, GERMANY.

## PROCESS FOR THE MANUFACTURE OF BLEACHED SOAP.

968,438.

Specification of Letters Patent. Patented Aug. 23, 1910.

No Drawing.

Application filed June 6, 1907. Serial No. 377,510.

*To all whom it may concern:*

Be it known that I, FRITZ WIEDERMANN, residing at 16 Friederich Karlplatz, Charlottenburg, Kingdom of Prussia, German Empire, have invented new and useful Improvements in Processes for the Manufacture of Bleached Soap, of which the following is a specification.

Heretofore it has been impossible to manufacture light colored soaps from dark or discolored oils, fatty acids, fats and resins. It was therefore necessary to subject the raw materials to a bleaching process before saponification. This presented the defect that special apparatus were necessary and that a long time was required for carrying the process into practice, thus rendering it considerably more costly. It is true that attempts have been made to bleach soaps after their formation by adding hypochlorite to the soap. This, however, imparted an unpleasant smell to the soap, and this smell was transmitted to the articles washed with it.

In the process forming the object of the present invention the bleaching is effected during the boiling of the soap, that is to say during the process of its manufacture. It has been found that the alkaline salts of persulfuric acid, without presenting the defects of chlorin bleaching, effect a bleaching during the saponification process, so that the final product is light colored. In particular the process has proved to be advantageous for linseed oil, cotton seed oil, neat's foot oil, palm oil and the low-graded olive-oil called sulfur oil.

The process is carried into practice by adding the alkaline salts of persulfuric acid, such for example as persulfate of sodium, to the soap during or after boiling, according to the color of the raw material and the

color desired for the final product. Generally the quantity of the persulfate used should amount to say  $\frac{1}{2}\%$  of the oil or fat. 45 A larger or a smaller proportion may, however, be used. The boiling operation is carried out in the usual manner.

By means of this process the great advantage is attained that losses such as would otherwise occur in bleaching oils and fats are avoided and that the products formed from the bleach during the bleaching operation, such for example as sulfate of sodium, sulfate of potassium and the like substances 55 do not impair the soap but on the contrary are of advantage to it. The alkaline salts employed are soluble in water.

The present process is particularly suited for soft soaps, which it has hitherto been 60 difficult to obtain in a clear condition.

Example: 2000 kgs. of red palm oil are boiled with 1200 kgs. of soda lye at 40° Baumé and the necessary water so as to form a thin jelly. Then 20 kgs. of sodium 65 persulfate are dissolved in 150 kgs. of water and added to the jelly, the whole being mixed and boiled until the red color has changed into a whitish yellow. Thereupon the graining is effected as usual. 70

I claim:

The process for the manufacture of bleached soap which consists in adding alkali salts of the persulfuric acids to the components of the soap after the beginning of 75 the saponification and before the end of the saponification.

In witness whereof I have hereunto signed my name this 17th day of May 1907, in the presence of two subscribing witnesses.

FRITZ WIEDERMANN.

Witnesses:

HENRY HASPER,  
WOLDEMAR HAUPT.